

## UNITED STATES PATENT OFFICE.

HENRY DREYFUS, OF LONDON, ENGLAND.

## MANUFACTURE OF ARTIFICIAL TEXTILE PRODUCTS.

No Drawing. Application filed May 26, 1923, Serial No. 641,760, and in Great Britain July 6, 1923.

This invention relates to the manufacture of artificial threads or filaments from solutions of cellulose acetate, or other organic esters of cellulose, ethyl or methyl cellulose 5 hereinafter all included in the term organic derivative of cellulose or other ethers of cellulose, by the evaporative or dry spinning method, that is to say wherein such solutions are spun into an evaporating atmosphere of air or other gas, and the threads or filaments solidify by evaporation of the solvent carried by the threads or filaments.

The invention is more particularly intended for the manufacture of threads or 15 filaments of cellulose acetate by such processes.

In dry spinning solutions of cellulose acetate or other organic cellulose esters or ethers such as referred to, in the solvents 20 commonly employed, such as acetone, methyl-ethyl ketone, methyl acetate, and so forth, the relatively high temperatures of the air or other gaseous current passed through the metiers or spinning casings to solidify the 25 filaments or threads, may tend to cause the filaments to set or shrink too suddenly or more or less irregularly, so that unevenness results in the resulting threads or filaments, and particularly when relatively dilute spinning 30 solutions are employed, especially when these are drawn out or produced under traction.

It has now been found that by employing spinning solutions of the cellulose acetate or 35 other organic derivatives of cellulose in or containing solvents of very low boiling points, the spinning can be effected at lower temperatures, and a more regular evaporation of the solvent from the solidifying filament can be obtained. Such very low boiling 40 solvents are for example acetaldehyde or formaldehyde. Mixtures of two or more of the very low boiling solvents may be employed. The mixtures may have a higher 45 solvent power for the cellulose derivative than the separate solvents.

The low boiling solvent or solvents are 50 preferably employed in association with the usual solvents or other solvents or liquids 55 having higher boiling points than the very low boiling solvents, as in this way, while a relatively low temperature may be employed for the evaporation of the filaments, uniform evaporation and formation of the filaments can take place so that they may draw 60 out to a more regular form. The low boil-

ing solvents may however be employed without such other solvents.

By way of example I may employ spinning solutions of cellulose acetate dissolved 60 in a mixture of acetone with acetaldehyde or formaldehyde (e. g. commercial formaldehyde solution), or with both acetaldehyde and formaldehyde (e. g. commercial formaldehyde solution). The proportion of the 65 acetone relatively to the acetaldehyde or other very low boiling solvent or solvents may vary according to requirement. Instead of acetaldehyde or formaldehyde, other solvents of the cellulose ester or ether 70 having very low boiling points may be employed; and instead of acetone other solvents of the cellulose ester or ether may be employed having higher boiling points than the 75 low boiling solvents.

With such mixtures the acetaldehyde, formaldehyde or other low boiling solvent or solvents may evaporate more rapidly than the acetone or other solvent or higher boiling point, so that a progressively decreasing rate of evaporation and consequent solidification of the filaments in their travel can take place, thereby facilitating the production of more regular filaments or threads.

According to the invention also, the liquid or liquids of very low boiling point and the liquid or liquids of higher boiling point need not necessarily be separately solvents of the cellulose ester or ether, provided that a mixture of them is a solvent therefor.

It has further been found that the formation of filaments or threads by the dry-spinning or evaporative method from solution of cellulose acetate or other cellulose esters or ethers in the very low boiling solvents or liquids such for instance as acetaldehyde or formaldehyde, or mixtures of them, can be improved by the addition or employment of water in said solution. Such addition, amongst other advantages, assists in controlling the speed of evaporation of the low boiling solvents in the solidification of the filaments and improves the regularity of the filaments produced. By way of example one may employ solutions of cellulose acetate in acetaldehyde or other very low boiling solvent, or mixtures of them, diluted with water to a desired or suitable extent, which should of course not be sufficient to precipitate the cellulose acetate but should 105 preferably be a mixture in such proportions as to give the best solvent power. The ex-

tent of dilution may be varied according to the temperature at which the filaments or threads are produced or other requirements.

It is to be understood that water may likewise be added to or employed in solutions of cellulose acetate or other cellulose esters or ethers in the low boiling liquid or liquids associated with the usual solvents or liquids or others having a higher boiling point than

10 the low boiling liquid or liquids.

The following are some examples of spinning solutions according to the invention, it being understood that these are given only by way of illustration and that the constitu-

15 ents and proportions may be varied widely without departing from the invention.

(1) Cellulose acetate is dissolved in acetaldehyde in quantity to form a 10-20% solution.

20 (2) A 10-20% solution of cellulose acetate is made in a mixture of acetaldehyde and acetone, the acetone amounting to from about one half to three fourths of the mixed solvent.

25 (3) A solution similar to (1) or (2) but having added to it about 5-10% of water calculated on the weight of the cellulose acetate.

The solutions may be spun at any suitable 30 temperatures, which may vary according to whether or not higher boiling solvents or liquids are employed together with the very low boiling solvents or liquids, and according to the amount of such higher boiling solvents or liquids. For example a solution in acetaldehyde alone may be spun at about ordinary atmospheric temperature, while solutions in mixtures of acetaldehyde and acetone, such as the solutions of example (2) 40 or (3), may be spun at somewhat higher temperatures, increasing with the percentage of acetone contained in them.

What I claim and desire to secure by Letters Patent is:—

45 1. Process for the production of artificial filaments or threads which consists in spinning into an evaporative atmosphere, a solution containing an organic derivative of cellulose in solution in a solvent liquid comprising a low boiling organic compound having a boiling point below 40° C.

50 2. Process for the production of artificial filaments or threads which consists in spinning into an evaporative atmosphere, a solution containing an organic derivative of cellulose in solution in a solvent liquid comprising a low boiling organic compound having a boiling point below 40° C. and a volatile liquid having a higher boiling point.

55 3. Process for the production of artificial filaments or threads which consists in spinning into an evaporative atmosphere, a solution containing an organic derivative of cellulose in solution in a solvent liquid comprising a low boiling organic compound hav-

ing a boiling point below 40° C, and a volatile organic liquid having a higher boiling point.

4. Process for the production of artificial 70 filaments or threads which consists in spinning into an evaporative atmosphere, a solution containing an organic derivative of cellulose in solution in a solvent liquid comprising a low boiling organic compound having a boiling point below 40° C. and a volatile organic liquid having a higher boiling point, and water.

5. Process for the production of artificial 80 filaments or threads which consists in spinning into an evaporative atmosphere, a solution containing an organic derivative of cellulose in solution in a solvent liquid comprising an aliphatic aldehyde having a boiling point not higher than about 21° C.

6. Process for the production of artificial 85 filaments or threads which consists in spinning into an evaporative atmosphere, a solution containing an organic derivative of cellulose in solution in a solvent liquid comprising an aliphatic aldehyde having a boiling point not higher than about 21° C., and a volatile liquid having a higher boiling point.

7. Process for the production of artificial 95 filaments or threads which consists in spinning into an evaporative atmosphere, a solution containing an organic derivative of cellulose in solution in a solvent liquid comprising an aliphatic aldehyde having a boiling point not higher than about 21° C., and a volatile organic liquid having a higher boiling point.

8. Process for the production of artificial 105 filaments or threads which consists in spinning into an evaporative atmosphere, a solution containing an organic derivative of cellulose in solution in a solvent liquid comprising an aliphatic aldehyde having a boiling point not higher than about 21° C., and a volatile organic liquid having a higher boiling point.

9. Process for the production of artificial 115 filaments or threads which consists in spinning into an evaporative atmosphere, a solution containing an organic derivative of cellulose in solution in a solvent liquid comprising acetaldehyde.

10. Process for the production of artificial 120 filaments or threads which consists in spinning into an evaporative atmosphere, a solution containing an organic derivative of cellulose in solution in a solvent liquid comprising acetaldehyde and a volatile liquid having a higher boiling point.

11. Process for the production of artificial 125 filaments or threads which consists in spinning into an evaporative atmosphere, a solution containing an organic derivative of cellulose in solution in a solvent liquid comprising acetaldehyde and acetone.

12. Process for the production of artificial filaments or threads which consists in spinning into an evaporative atmosphere, a solution containing an organic derivative of cellulose in solution in a solvent liquid comprising acetaldehyde and acetone and water.
13. Process for the production of artificial filaments or threads which consists in spinning into an evaporative atmosphere, a solution containing cellulose acetate in solution in a solvent liquid comprising a low-boiling organic compound having a boiling point below 40° C.
14. Process for the production of artificial filaments or threads which consists in spinning into an evaporative atmosphere, a solution containing cellulose acetate in solution in a solvent liquid comprising a low-boiling organic compound having a boiling point below 40° C. and a volatile liquid having a higher boiling point.
15. Process for the production of artificial filaments or threads which consists in spinning into an evaporative atmosphere, a solution containing cellulose acetate in solution in a solvent liquid comprising a low-boiling organic compound having a boiling point below 40° C. and a volatile organic liquid having a higher boiling point.
16. Process for the production of artificial filaments or threads which consists in spinning into an evaporative atmosphere, a solution containing cellulose acetate in solution in a solvent liquid comprising a low-boiling organic compound having a boiling point below 40° C. and a volatile organic liquid having a higher boiling point and water.
17. Process for the production of artificial filaments or threads which consists in spinning into an evaporative atmosphere, a solution containing cellulose acetate in solution in a solvent liquid comprising an aliphatic aldehyde having a boiling point not higher than about 21° C.
18. Process for the production of artificial filaments or threads which consists in spinning into an evaporative atmosphere, a solution containing cellulose acetate in solution in a solvent liquid comprising an aliphatic aldehyde having a boiling point not higher than about 21° C. and a volatile liquid having a higher boiling point.
19. Process for the production of artificial filaments or threads which consists in spinning into an evaporative atmosphere, a solution containing cellulose acetate in solution in a solvent liquid comprising an aliphatic aldehyde having a boiling point not higher than about 21° C. and a volatile organic liquid having a higher boiling point.
20. Process for the production of artificial filaments or threads which consists in spinning into an evaporative atmosphere, a solution containing cellulose acetate in solution in a solvent liquid comprising an aliphatic aldehyde having a boiling point not higher than about 21° C. and a volatile organic liquid having a higher boiling point.
21. Process for the production of artificial filaments or threads which consists in spinning into an evaporative atmosphere, a solution containing cellulose acetate in solution in a solvent liquid comprising acetaldehyde.
22. Process for the production of artificial filaments or threads which consists in spinning into an evaporative atmosphere, a solution containing cellulose acetate in solution in a solvent liquid comprising acetaldehyde and a volatile liquid having a higher boiling point.
23. Process for the production of artificial filaments or threads which consists in spinning into an evaporative atmosphere, a solution containing cellulose acetate in solution in a solvent liquid comprising acetaldehyde and a volatile organic liquid having a higher boiling point.
24. Process for the production of artificial filaments or threads which consists in spinning into an evaporative atmosphere, a solution containing cellulose acetate in solution in a solvent liquid comprising acetaldehyde and acetone.
25. Process for the production of artificial filaments or threads which consists in spinning into an evaporative atmosphere, a solution containing cellulose acetate in solution in a solvent liquid comprising acetaldehyde and a volatile organic liquid having a higher boiling point and water.

In testimony whereof I have hereunto subscribed my name.

HENRY DREYFUS.